

1

3,230,159

## ACIDIC TIN-PLATING PROCESS

Shigeru Yonezaki, Yawata, Fukuoka, Hazime Nitto, Ozawa-machi, Tobata, Fukuoka, and Hidejiro Asano, Tobata, Fukuoka, Japan, assignors to Yawata Iron & Steel Co., Ltd., Tokyo, Japan, a corporation of Japan  
No Drawing. Filed Oct. 15, 1962, Ser. No. 230,695

Claims priority, application Japan, Oct. 20, 1961,  
36/37,703

6 Claims. (Cl. 204—54)

This invention relates to improvements in an acidic tin-plating process.

Acidic tin-plating processes are most extensively adopted in producing electroplated tin plates.

Generally, in acidic tin plating, the electrolytic plating bath consists mostly of sulphuric acid, phenol sulphonic acid, tin sulphate and a tin halide with the addition thereto of a proper additive such as, for example, diphenylol propane. However, such known additive has a drawback that its solubility in an acidic plating bath is so low that it can hardly be used.

We have confirmed that a naphthylamine represented by the general formula:



(wherein R is hydrogen or a residue of a hydrocarbon compound having 1 to 5 carbon atoms) and its derivatives are very high in solubility in an acidic tin-plating bath and that, when said compound is added in an amount of at least about 0.1 g./l. to a plating bath, a beautiful smooth electrodeposit will be obtained on the surface of a strip.

Naphthylamine and its derivatives are very high in solubility in an acidic bath as the common property of amino compounds and can remarkably increase the workability. But, below the above mentioned concentration of 0.1 g./l., no desired effect can be expected.

The number of the carbon atoms of the residue of the hydrocarbon compound bonded with the nitrogen atom of the naphthylamine or its derivative is limited to 1 to 5. If it is more than 6, the solubility in the acidic bath will be reduced and it will not be desirable for industrial practice.

The luster of the electrodeposited tin plate according to the present invention is considered to be due to the fact that the N of the amino radical of the naphthylamine or its derivative will be adsorbed at the forward end of electrodeposited tin, the large atomic group of nonreactive naphthalene will prevent any later electrodeposition and a smooth electrodeposited surface will be obtained.

The naphthylamine derivatives to be used in the present invention are enumerated, for example, as follows:



2



The present invention shall be explained with reference to examples. However, the scope of the present invention is not intended to be limited to these examples.

## Example 1

| Composition of the plating bath: | G./l. |
|----------------------------------|-------|
| Phenol sulphonic acid            | 25    |
| Tin sulphate                     | 30    |
| N-ethyl- $\alpha$ -naphthylamine | 2     |

Electric current densities: 1 a./dm.<sup>2</sup>, 5 a./dm.<sup>2</sup> and 10 a./dm.<sup>2</sup>

Temperature: 40° C.

Thicknesses of the plating: 0.25 lb./bb., 0.5 lb./bb. and 1.00 lb./bb.

## Example 2

A plating bath in which 2 g./l. of N-ethyl- $\alpha$ -naphthylamine in Example 1 were replaced with 2 g./l. of  $\alpha$ -naphthylamine was used.

## Example 3

A plating bath in which 2 g./l. of N-ethyl- $\alpha$ -naphthylamine in Example 1 were replaced with 2.5 g./l. of N-methyl- $\alpha$ -naphthylamine was used.

## Example 4

| Composition of the bath:        | G./l. |
|---------------------------------|-------|
| Phenol sulphonic acid           | 25    |
| Tin sulphate                    | 60    |
| N-ethyl- $\beta$ -naphthylamine | 2     |

Current densities: 5 a./dm.<sup>2</sup>, 10 a./dm.<sup>2</sup> and 20 a./dm.<sup>2</sup>

Temperature: 40 to 60° C.

Thickness of the plating: 0.25 to 1.00 lb./bb.

## Example 5

A plating bath in which 2 g./l. of N-ethyl- $\beta$ -naphthylamine in Example 4 were replaced with 2 g./l. of  $\beta$ -naphthylamine was used.

When the composition was electrodeposited on a strip under the above mentioned conditions, a tin plate having a milk-white lustrous surface was obtained. When this plate was subjected to a tin-melting treatment by direct electric heating, a favorable plate was obtained.

Even when the composition of the plating bath in the process of the present invention is varied in a range con-

3

siderably wider than the above mentioned compositions, a lustrous surface can be obtained.

What we claim is:

1. In a process for producing electroplated tin plate in an acidic tin-plating bath containing an additive, the improvement wherein the additive is a naphthylamine of the formula



wherein R is a member selected from the group consisting of H and alkyl with 1 to 5 carbon atoms, in an amount of at least about 0.1 g./l.

2. In a process for producing electroplated tin plate in an acidic tin-plating bath, the improvement wherein the tin plating is effected in the presence in the acidic bath of at least 0.1 g./l. of a naphthylamine of the formula

4



wherein R is a member selected from the group consisting of H and alkyl with 1 to 5 carbon atoms.

3. An improvement according to claim 1, wherein the naphthylamine is N-ethyl- $\alpha$ -naphthylamine.  
 10 4. An improvement according to claim 1, wherein the naphthylamine is  $\alpha$ -naphthylamine.  
 5. An improvement according to claim 1, wherein the naphthylamine is N-ethyl- $\beta$ -naphthylamine.  
 15 6. An improvement according to claim 1, wherein the naphthylamine is  $\beta$ -naphthylamine.

#### References Cited by the Examiner

##### UNITED STATES PATENTS

|    |           |         |          |       |        |
|----|-----------|---------|----------|-------|--------|
| 20 | 2,446,716 | 8/1948  | Nachtman | ----- | 204-43 |
|    | 2,450,794 | 10/1948 | Harris   | ----- | 204-54 |
|    | 2,552,920 | 5/1951  | Allen    | ----- | 204-54 |
|    | 2,598,486 | 5/1952  | Andrews  | ----- | 204-54 |

JOHN H. MACK, Primary Examiner.